

# United States Patent [19]

Sobue et al.

[11] 3,902,897

[45] Sept. 2, 1975

[54] **HIGH HARDNESS SPHEROIDAL GRAPHITE  
CAST IRON**

[75] Inventors: **Masahisa Sobue, Tokyo; Toshimi  
Sasaki, Abiko, both of Japan**

[73] Assignee: **Hitachi, Ltd., Japan**

[22] Filed: **Jan. 4, 1974**

[21] Appl. No.: **430,762**

[30] **Foreign Application Priority Data**

Jan. 12, 1973 Japan ..... 48-5983

[52] **U.S. Cl. 75/124; 75/123 CB; 75/123 J;  
75/123 K; 148/35**

[51] **Int. Cl. C22c 37/10**

[58] **Field of Search 75/123 CB, 124, 124 J,  
75/123 K; 148/35**

[56] **References Cited**

UNITED STATES PATENTS

2,485,761 10/1949 Millis ..... 75/123 CB

|           |        |                  |           |
|-----------|--------|------------------|-----------|
| 2,501,059 | 3/1950 | Kluijtmans ..... | 75/123 CB |
| 2,516,524 | 7/1950 | Millis .....     | 75/123 CB |
| 2,749,238 | 6/1956 | Millis .....     | 75/123 CB |

*Primary Examiner*—L. Dewayne Rutledge

*Assistant Examiner*—Arthur J. Steiner

*Attorney, Agent, or Firm*—Craig & Antonelli

[57]

## ABSTRACT

This invention is characterized in that 1.5 – 6.0% of Ni, 0.2 – 2.0% of Al and 0.1 – 1.0% of Mo are added to the general spheroidal graphite cast iron. Thus obtained spheroidal graphite cast iron has the following characteristics: it has low hardness in its cast state (as cast) and hence can easily be mechanically worked; the hardness is greatly increased by the subsequent heat treatment; and substantially no deformation is caused with the heat treatment.

**6 Claims, 3 Drawing Figures**

PATENTED SEP. 2 1975

3,902,897

FIG.1



FIG.2



FIG.3



# HIGH HARDNESS SPHEROIDAL GRAPHITE CAST IRON

## BACKGROUND OF THE INVENTION

This invention relates to a spheroidal graphite cast iron and more particularly it relates to a spheroidal graphite cast iron having a high wear resistance and mechanical workability.

Wear resistance of the usual spheroidal graphite cast iron is improved with increase in hardness. Therefore, conventionally the hardness is increased by induction hardening, oil hardening or water hardening.

However, according to these methods, quenching cracks and strains are apt to be caused because the iron is once heated to a high temperature. Furthermore, in case of high accuracy in size being desired, mechanical working is required after heat treatment and thus the operating steps are increased and the cost becomes higher. Moreover, in many cases, the spheroidal graphite cast iron is cast into products of complicated shapes and it is sometimes impossible to subject these products to said heat treatment.

## OBJECT OF THE INVENTION

The object of this invention is to provide a spheroidal graphite cast iron which has the following characteristics: the as-cast iron has low hardness and mechanical working can easily be accomplished; subsequently, the hardness is greatly increased by a heat treatment at a relatively low temperature; and deformation caused by heat treatment is very small.

## SUMMARY OF THE INVENTION

The spheroidal graphite cast iron of this invention comprises, by weight, 2.3 - 4.2 % of C, 1.5 - 5.0 % of Si, not more than 1.0 % of Mn, not more than 0.1 % of spheroidizing element, 1.5 - 6.0 %, preferably about 2.7 % of Ni, 0.1 - 1.0 %, preferably about 0.5 % of Mo, 0.1 - 1.0 %, preferably 0.5 - 1.0 % of Al and the balance of Fe and incidental impurities.

Furthermore, according to this invention, the cast iron having the above compositions is subjected to tempering treatment.

## BRIEF DESCRIPTION OF DRAWING

FIG. 1 and FIG. 2 are rough front and side views which explain the condition of abrasion test carried out in this invention, respectively.

FIG. 3 is a drawing which explains measurement of change in size.

## DESCRIPTION OF THE PREFERRED EMBODIMENTS

The following examples show that according to this invention a spheroidal graphite cast iron which has a low hardness and a high mechanical workability in as-cast state, hardness of which is greatly increased by 10 subsequent heat treatment and which shows little deformation caused by heat treatment can be obtained.

Various spheroidal graphite cast irons having compositions as shown in Table 1 were produced by casting in a keel block mold of 30 mm in thickness. Then, test 15 pieces were taken and were subjected to tempering treatment at 500°C for 4 hours. The test pieces of the cast irons before subjected to the tempering treatment and after subjected to the tempering treatment were subjected to Brinell hardness test and abrasion test. 20 The results are shown in Table 2. Moreover, changes in size caused by the tempering treatment were measured and the results are shown in Table 2.

Said abrasion test was carried out using the Ogoshi abrasion tester [See "Collection of Articles of Japan 25 Mechanical Society" (Vol. 21, pages 555 - , 1955) by Ogoshi et al] under the following conditions: load . . . . 6.5 kg, abrasion speed . . . . 0.5 m/s and abrasion distance . . . . 200 m. The test method is as follows: As shown in FIGS. 1 and 2, revolving ring 2 (outer diameter 30 φ) made of sample No. 1 in Table 1 was pressed against a fixed test piece 1 whose wear resistance is to be measured at dried state and it was revolved. Abraded width . . . in the fixed test piece 1 was measured and wear resistance was compared on the basis of 35 this value.

Measurement of changes in size due to the tempering treatment was effected by measuring length L of the test pieces before and after subjected to tempering treatment as shown in FIG. 3 and expressing the change 40 in the length by percentage.

In Table 1, Sample No. 1 is the conventional spheroidal graphite cast irons, comparative samples No. 2 - 4 are the cast irons containing Ni and either one of Al or Mo and samples No. 5 - 17 are the spheroidal graphite 45 cast irons of this invention.

Table 1

| No. | Chemical Compositions (%) |      |      |       |      |       |      |         |
|-----|---------------------------|------|------|-------|------|-------|------|---------|
|     | C                         | Si   | Mn   | Mg    | Ni   | Al    | Mo   | Fe      |
| 1   | 3.35                      | 2.50 | 0.33 | 0.051 | —    | —     | —    | Balance |
| 2   | 3.20                      | 2.45 | 0.40 | 0.049 | 3.10 | 0.501 | —    | "       |
| 3   | 3.22                      | 2.55 | 0.40 | 0.051 | 2.72 | —     | 0.51 | "       |
| 4   | 3.17                      | 2.40 | 0.36 | 0.050 | 4.01 | —     | 0.19 | "       |
| 5   | 3.20                      | 2.70 | 0.35 | 0.050 | 1.55 | 0.513 | 0.81 | "       |
| 6   | 3.31                      | 2.70 | 0.35 | 0.048 | 2.73 | 0.203 | 0.52 | "       |
| 7   | 3.35                      | 2.01 | 0.24 | 0.052 | 2.73 | 0.499 | 0.52 | "       |
| 8   | 3.20                      | 2.01 | 0.20 | 0.051 | 2.75 | 1.020 | 0.53 | "       |
| 9   | 3.25                      | 2.00 | 0.28 | 0.050 | 2.69 | 2.000 | 0.52 | "       |
| 10  | 3.18                      | 2.35 | 0.30 | 0.052 | 4.01 | 0.217 | 0.20 | "       |
| 11  | 3.54                      | 2.33 | 0.36 | 0.050 | 4.05 | 0.511 | 0.19 | "       |
| 12  | 3.20                      | 2.44 | 0.32 | 0.049 | 4.08 | 0.990 | 0.18 | "       |
| 13  | 3.55                      | 2.51 | 0.37 | 0.050 | 4.10 | 0.198 | 0.52 | "       |
| 14  | 3.55                      | 2.60 | 0.51 | 0.050 | 4.07 | 0.492 | 0.49 | "       |
| 15  | 3.60                      | 2.67 | 0.36 | 0.050 | 4.11 | 1.050 | 0.53 | "       |
| 16  | 3.15                      | 2.45 | 0.20 | 0.049 | 6.02 | 1.050 | 0.15 | "       |
| 17  | 3.27                      | 2.70 | 0.20 | 0.051 | 5.98 | 1.980 | 0.13 | "       |

Table 2

| No. | Brinell hardness |                  | Abraded width l (mm) |                  | Changes in size after tempering (%) |
|-----|------------------|------------------|----------------------|------------------|-------------------------------------|
|     | As-cast          | After* tempering | As-cast              | After* tempering |                                     |
| 1   | 188              | 187              | 4.01                 | 4.10             | 0.003                               |
| 2   | 262              | 257              | 1.99                 | 2.19             | 0.006                               |
| 3   | 317              | 325              | 0.85                 | 0.85             | 0.010                               |
| 4   | 350              | 356              | 0.55                 | 0.45             | 0.007                               |
| 5   | 250              | 265              | 2.00                 | 1.90             | 0.008                               |
| 6   | 268              | 326              | 1.88                 | 1.10             | 0.006                               |
| 7   | 283              | 370              | 1.27                 | 0.30             | 0.008                               |
| 8   | 275              | 363              | 1.33                 | 0.35             | 0.007                               |
| 9   | 280              | 363              | 1.27                 | 0.36             | 0.010                               |
| 10  | 331              | 352              | 0.65                 | 0.42             | 0.005                               |
| 11  | 321              | 354              | 0.85                 | 0.43             | 0.007                               |
| 12  | 321              | 352              | 1.05                 | 0.43             | 0.006                               |
| 13  | 352              | 363              | 0.43                 | 0.35             | 0.007                               |
| 14  | 331              | 375              | 0.79                 | 0.29             | 0.006                               |
| 15  | 325              | 388              | 0.70                 | 0.28             | 0.007                               |
| 16  | 354              | 390              | 0.40                 | 0.25             | 0.010                               |
| 17  | 343              | 395              | 0.44                 | 0.25             | 0.009                               |

\*500°C × 4 hours

It is clear from Table 2 that in case of the conventional spheroidal graphite cast iron No. 1 and No. 2 which had the compositions of No. 1 to which Ni and Al were added, hardness was not increased and rather slightly softened after subjected to tempering treatment. Furthermore, in case of samples No. 3 and 4 which had the compositions of sample No. 1 to which Ni and Mo were added, hardness was only slightly increased. Thus, in case of samples No. 1 – 4, substantially no change in hardness was caused before and after tempering treatment. Therefore, abraded width

hardly changed before and after tempering treatment and no improvement in wear resistance was recognized.

On the other hand, hardnesses of samples No. 5 – 17 of this invention were all increased after tempering treatment and the abraded width after tempering treatment was reduced as compared with those which were not subjected to the tempering treatment. Thus, it was confirmed that wear resistance was improved. This fact indicates that the spheroidal graphite cast iron of this invention has excellent mechanical workability in as-cast state and has a wear resistance after subjected to tempering treatment. Furthermore, from the fact that the change in length before and after tempering treatment was only a little and could be practically ignored as in Table 2, it was also confirmed that if the cast iron of this invention is previously subjected to finish working after casting, it can be used nearly as it is after tempering treatment.

Therefore, since the spheroidal graphite cast iron of this invention can easily be mechanically worked in as-cast state, and the hardness can be increased by the subsequent heat treatment to improve wear resistance. Furthermore, since the change in size caused by the heat treatment is such that may be ignored, the cast iron of this invention can be used as it is as various articles.

Reasons for limitation of the composition ranges of the elements in the spheroidal graphite cast iron of this invention are as follows:

C is essential for forming graphite and when content of C is less than 2.3 %, castability is lowered and simul-

taneously carbide is produced and when more than 4.2 %, strength is decreased. Therefore, content of C is limited to 2.3 – 4.2 %. Si is an important element which accelerates the graphitization and promotes decrease in eutectic carbon. When content of Si is less than 1.5 %, it has no graphitization accelerating effect and when more than 5.0 %, the iron becomes extremely brittle. Therefore, content of Si is limited to 1.5 – 5.0 %. When content of Mn which increases the strength exceeds 1.0 %, graphitization is obstructed and carbide is formed to make the iron brittle. Therefore, content of Mn is limited to not more than 1.0 %. The spheroidizing element such as Mg or Ca is added for spheroidization of graphite and when content thereof is more than 0.1 %, soundness of castings is damaged. Thus, the content is limited to not more than 0.1 %. As the spheroidizing elements, any of the known spheroidizing elements, for example, Mg, Ca, Ce, Mg–Ca, Mg–Ce, Mg–Ca–Ce, etc., may be used. When content of Ni which is essential for hardening is less than 1.5 %, hardening cannot be accomplished and when more than 6.0 %, martensite is produced in a large amount in as-cast state to result in too high hardness. Therefore, content of Ni is limited to 1.5 – 6.0 %. Al is essential in that it lowers hardness of iron in as-cast state and increases the hardness after heat treatment. When content of Al is less than 0.2 %, said effects cannot be attained and when more than 2.0 %, spheroidization of graphite is restrained and fluidity of melt is extremely lowered. Therefore, content of Al is limited to 0.2 – 2.0 %. Mo increases hardness after heat treatment and simultaneously shortens the time required for hardening and furthermore, addition of Mo can reduce the amount of Al which lowers fluidity of melt. However, when content of Mo is less than 0.1 %, the above effects cannot be attained and when more than 1.0 %, a large amount of carbide is formed in as-cast state to result in too high hardness. Therefore, content of Mo is limited to 0.1 – 1.0 %.

What is claimed is:

1. A high hardness spheroidal graphite cast iron which consists essentially of, on the basis of weight, 2.3–4.2% of C, 1.5 – 5.0% of Si, not more than 1.0% of Mn, not more than 0.1% of spheroidizing element, 1.5–6.0% of Ni, 0.2 – 2.0% of Al, 0.1–1.0% of Mo and the balance Fe and incidental impurities.
2. A spheroidal graphite cast iron according to claim 1, wherein content of Ni is about 2.7 %, that of Al is 0.5 – 1.0 % and that of Mo is about 0.5 %.
3. A spheroidal graphite cast iron according to claim 1, which is subjected to tempering treatment after casting to increase its hardness.
4. A spheroidal graphite cast iron according to claim 3, wherein said tempering treatment is at 500°C. for 4 hours.
5. A spheroidal graphite cast iron according to claim 1, wherein said spheroidizing element is Mg, Ca, Ce, Mg–Ca, Mg–Ce, or Mg–Ca–Ce and the amount of said spheroidizing element added is sufficient for spheroidization of graphite.
6. A spheroidal graphite cast iron according to claim 1, wherein said spheroidizing element is Mg and the content of Mg is from 0.048 to not more than 0.1%.